

June 10, 1947.

W. L. KEENE ET AL

2,421,891

COMPOSITE BILLET AND MANUFACTURE THEREOF

Filed March 18, 1943

Fig. 1.



Fig. 2.



Fig. 3.



INVENTORS

Walter L. Keene and  
William A. Carlson

by *Sabbing and Beers*  
*as attorneys*

## UNITED STATES PATENT OFFICE

2,421,891

COMPOSITE BILLET AND MANUFACTURE  
THEREOF

Walter L. Keene, Dormont, and William A. Carlson, Pittsburgh, Pa., assignors to Superior Steel Corporation, Pittsburgh, Pa., a corporation of Virginia

Application March 18, 1943, Serial No. 479,588

8 Claims. (Cl. 29—187.5)

1

This invention relates to composite billets and the manufacture thereof. It relates more particularly to the making of composite billets by assembling a plurality of metal members in such manner that when the billet is rolled strip of desired characteristics is produced.

The art of making composite billets is an old one. United States Patent No. 685,758 shows the making of a bimetallic billet by producing a flanged backing member of steel, applying to opposite faces of the flanged backing member facing members of copper and turning the flanges of the steel backing member down against the edges of the copper facing members to hold the latter in place. Various improvements have been made in the invention disclosed in this early patent, a number of the more recent and commercially important improvements being disclosed and claimed in copending applications owned by our assignee, Superior Steel Corporation. A number of the recent improvements have been made in connection with the development of strip consisting of steel clad on both sides with gilding metal for the manufacture of ammunition components such as bullet jackets.

Heretofore in the manufacture of composite billets by the application of facing members to a flanged backing member and the holding of the facing members in place by the flanges of the backing member it has been considered important that the flanges of the backing member closely embrace the edges of the facing members so as to hold them firmly in position. However, we have discovered that close embracement of the edges of the facing members by the flanges of the backing member is not always desirable and indeed in some instances is definitely undesirable. Difficulty has been encountered in the making and rolling of bimetallic billets by reason of the entry of air between the backing and facing members during heating and/or rolling which prevents proper bonding and results in the production of virtually worthless strip. This condition has been found to exist, for example, in the making of silver clad steel strip. The difficulty apparently arises through the relatively great differential expansion of silver over steel upon heating, which causes the silver facing members of the bimetallic billet, whose edges are closely confined by the flanges of the steel backing member, to bow up slightly, allowing the entry of air. We have found that this difficulty incident to the making and rolling of composite billets comprising a flanged backing member with facing members held in place by the flanges of

2

the backing member can be overcome by providing a space between at least one edge of each facing member and the laterally adjacent portion of the flange cooperating with such edge. Desirably such spaces may be provided at both edges of the facing members. The provision of such space or spaces allows for substantial differential expansion between the facing members and the backing member and we find that when such spaces are provided no difficulty is encountered with bowing up of the facing members during heating and/or rolling and consequent entry of air between the backing member and facing members.

15 The provision of the space or spaces just mentioned is also of advantage generally in the making and rolling of composite billets as it allows room for slight minor adjustments of position between the backing member and facing members 10 during rolling without imposing substantial strains on the billet components, even though there were no differential expansion.

20 In the making of composite billets comprising a flanged backing member with facing members held in place thereon by the flanges thereof it has heretofore been customary to produce the flanged billet components or backing members by rolling. This method of production has advantages, particularly in quantity production of a 25 standardized item, as large numbers of flanged backing members can be more economically produced by rolling than otherwise. However, the production of the flanged backing members by rolling has certain disadvantages which prior to the present invention have not been overcome. 30 It is difficult to produce by rolling flanged backing members above certain widths, so if exceptionally wide strip is desired the cost of the backing members is high out of proportion. Moreover, if very narrow strip is to be produced either 35 special flanged billet components must be rolled, necessitating an outlay for special rolls, or strip made from relatively wide billets must be slit. In the latter case there is considerable waste 40 unless the width of the strip produced by the wider billet is substantially an exact multiple of the width of the narrower strip desired.

45 Moreover, the metal comprising the flanges of the flanged component of a composite billet constitutes a substantial part of the metal of the component as a whole and when such a component is made by rolling the flanges must be of the same metal as the body of the component. If the body of the component is of a relatively 50 costly metal the making of the flanges out of the

same metal unnecessarily increases the cost of the billet as the flanges do not form part of the finished strip but are sheared off after rolling.

We have overcome all of the disadvantages above outlined which are inherent in the use of rolled flanged billet components. We provide a flanged billet component which is not rolled but which comprises a body portion which may be in the form of an ordinary plate or rectangular rolled section with flanges attached thereto by welding or other means. Such a component has great advantages in economy and flexibility. By selecting a body portion of suitable width and welding the opposed flanges thereto at or adjacent its edges a "tailor made" backing member may be produced which will avoid any scrap loss other than the shearing off of the flanges, which always occurs. The flanges may be of metal different from the metal of the body portion of the component.

We have found that when a space or spaces is or are to be left between one or both of the flanges of a flanged backing member and an edge or edges of a facing member to be held in place against the backing member by the flanges, the flanges should have their extremities extending generally toward one another before the facing member is applied so that after the facing member is applied the extremities of the flanges can be forced down against the outer surface of the facing member to hold it in place while still leaving the spaces at the lateral edges of the facing member. Our invention is of particular value in such circumstances as the production by rolling of a flanged billet component with the extremities of the opposed flanges extending generally toward one another prior to application of a facing member therebetween is economically impossible and the formation of overhung flanges by machining is virtually in the same category. We solve the problem in a most simple and effective way by welding or similarly fastening to the body portion of the component flange members having their extremities extending generally toward one another. Such flange members are preferably of angular or L shape. Thus our invention is of importance both in relation to the feature of providing space between a facing member and the flanges of a backing member to which it is connected and also in relation to the economical manufacture of various widths of strip and the economical manufacture of strip using a billet the body portion of whose flanged backing member is of relatively expensive metal.

Other details, objects and advantages of the invention will become apparent as the following description of certain present preferred embodiments thereof and certain present preferred methods of practicing the same proceeds.

In the accompanying drawings I have shown certain present preferred embodiments of the invention and have illustrated certain present preferred methods of practicing the same, in which

Figure 1 is a vertical transverse cross-sectional view through components of a composite billet assembled ready for final fastening together;

Figure 2 is a fragmentary vertical transverse cross-sectional view similar to the left-hand portion of Figure 1 showing the inwardly directed extremity of one of the flanges which are welded to the body of the backing member pressed down against the outer surface of the facing member to hold it in place; and

Figure 3 is a fragmentary vertical transverse cross-sectional view similar to the left-hand por-

tion of Figure 1 but showing a modified structure.

Referring now more particularly to the drawings, there is shown in Figures 1 and 2 a backing member designated generally by reference numeral 2 and which comprises a body portion 3 and flanges 4, together with a facing member 5. Only two flanges are shown, but it is to be understood that the flanges shown at the top of Figure 1 may be duplicated at the bottom so that strip faced or clad both top and bottom may be made. Since the manner of attaching the bottom facing member would be the same as the manner of attaching the top facing member the bottom flanges and facing member are omitted from the drawings for simplicity.

The body portion 3 of the backing member 2 may be a plate or rolled section of steel or other metal of desired characteristics. In the form shown it is of rectangular vertical cross section and uniform cross section throughout its length so may and ordinarily will be a rolled section. The flanges 4 are not formed integral with the body portion 3 by rolling but are fastened to the body portion, as by welding. Welding material 6 is shown positioned in the exterior corners between the body portion and the flanges whereby the flanges are strongly held in place and become in effect integral portions of the backing member 2. The flanges 4 are shown as of angular or inverted L shape with their extremities 7 extending generally toward one another. Initially the flange extremities are spaced from the upper surface of the body portion 3 sufficiently to allow the facing member 5 to be freely inserted longitudinally between the flanges. Ordinarily the facing member will be thus inserted as the inturned flange extremities would probably interfere with insertion of the facing member in any other way.

The flanges 4 may be of metal similar to or dissimilar from the metal of the body portion 3, one advantage of the structure shown being that if the body portion 3 is made of relatively expensive metal the cost can be reduced by using flanges of relatively inexpensive metal where as with an integral rolled flanged section the flanges are of necessity of the same metal as the body portion. Likewise the attaching of the flanges to the body portion by welding makes it feasible to employ flanges with inturned extremities which could not economically or practicably be employed in integral rolled sections. The employment of such flanges in turn makes feasible the provision of spaces 8 between the lateral edges of the facing member 5 and the portions of the flanges below the extremities thereof as clearly shown in Figure 1. If the flanges simply stood up straight prior to being deformed to hold the facing member in place it would be virtually impossible to turn them down about the edges of the facing member and still leave the spaces 8 whose advantages we have pointed out above. Satisfactory results may ordinarily be obtained by the provision of a space 8 at one edge only of the facing member, although we prefer to provide such spaces at both edges. If only one space is provided it should be twice as wide as each space if two are provided. The width of the space or spaces between the edges of the facing member and the portions of the flanges of the backing member opposite the edges of the facing member should be determined to allow for whatever relative expansion will occur when the billet is heated to hot rolling temperature and rolled, taking into

consideration the coefficients of expansion of the metals employed.

After the members 2 and 5 are assembled as shown in Figure 1 the flange extremities 7 are pressed or peined down against the outer surface of the facing member 5 as shown in Figure 2. This may be done by rolling or otherwise. By reason of the fact that the extremities of the flanges extend generally toward one another prior to their being deformed to hold the facing member, the facing member can be held in place without eliminating the spaces 8.

The welded joints formed between the body portion 3 and the flanges 4 as shown in Figures 1 and 2 are exceptionally strong as the welding material 6 lies in the longitudinally extending corner between the upper surface of the body portion 3 and the outer surface of each flange. By positioning the welding material 6 at the outside of each flange it does not interfere with the cooperative relationship between the flanges and the facing member 5.

Figure 3 shows a modified form of structure in which parts corresponding to the parts shown in Figures 1 and 2 are identified with the same reference numerals but each with a prime affixed. The difference between the structure of Figure 3 and that of Figure 1 is that in Figure 3 the body portion 3' of the backing member 2' is somewhat narrower than in Figure 1, the flanges 4' being positioned flush with the edges of the body portion 3' and the welding material 6' spanning the upper edge of the body portion. This does not make as strong a weld as in the structure of Figure 1 but it results in some saving of material. One or the other of the forms shown may be of advantage under different circumstances.

The metals employed for the body portion of the backing member, the flanges and the facing member may be selected to meet particular conditions. If the flanges are welded to the body portion both the body portion and the flanges must be of weldable metal. Purely by way of example, the body portion may be of low or high carbon steel, Austenitic manganese steel, stainless steel, copper, etc. The facing or cladding metal may be any metal which can be bonded to the backing metal to produce a bimetallic strip. For example, the facing metal may be of gilding metal, stainless steel, copper, silver, etc. Likewise the flanges may be of any suitable metal, but since their function is simply to hold the facing or cladding metal in place during rolling and they are afterwards sheared off they are ordinarily of the cheapest low carbon steel.

A further advantage of the invention is that the backing member may be made on non-machinable steel, such, for example, as Hadfield manganese steel. It would not be possible using such a steel to produce the flanges with turned extremities by machining.

A further advantage of the invention is that if the body portion of the backing member is made of high carbon steel and the flanges are made of low carbon steel no annealing of the flanges prior to deformation thereof against the facing member is necessary as might be the case if the entire backing member including the flanges were rolled or otherwise formed of high carbon steel. Annealing of the flanges would in all likelihood be necessary if they were of high carbon steel and rolled integrally with the body portion of the backing member so that they would stand straight up and have to be subjected to a relatively great amount of work in being turned

or peined over against the facing member. This further shows the advantage of using the angular or L-shaped flanges.

Another advantage incident to the use of flanges on the backing member whose extremities extend generally toward one another prior to peining is that the peining or pressing of the flanges down against the facing member may be accomplished by ordinary cylindrical rolls and special rolls are not necessary as is the case when the flanges have to be turned laterally and downwardly from an initially upright position.

While we have shown and described certain present preferred embodiments of the invention and certain present preferred methods of practicing the same it is to be distinctly understood that the invention is not limited thereto but may be otherwise variously embodied and practiced within the scope of the following claims.

We claim:

1. A composite billet comprising a metallic backing member, opposed generally L-shaped flanges welded to the backing member with one leg of each flange extending generally at right angles to a face of the backing member and having its extremity butting against said face and with the other legs of the flanges extending toward each other and a metallic facing member disposed against said face of the backing member between the first mentioned legs of the flanges with the second mentioned legs of the flanges overlying a minor portion thereof and held in place against the backing member by the flanges.
2. A composite billet comprising a metallic backing member, opposed generally L-shaped flanges welded to the backing member with one leg of each flange extending generally at right angles to a face of the backing member and having its extremity butting against said face and with the other legs of the flanges extending toward each other and a metallic facing member disposed against said face of the backing member between the first mentioned legs of the flanges with the second mentioned legs of the flanges overlying a minor portion thereof, spaced from at least one of said first mentioned legs and held in place against the backing member by the flanges.
3. A composite billet comprising a metallic backing member, opposed generally L-shaped flanges welded to the backing member with one leg of each flange extending generally at right angles to a face of the backing member and having its extremity butting against said face and with the other legs of the flanges extending toward each other and a metallic facing member disposed against said face of the backing member between the first mentioned legs of the flanges with the second mentioned legs of the flanges overlying a minor portion thereof and held in place against the backing member by the second mentioned legs only of the flanges.
4. A composite billet comprising a metallic backing member, opposed generally L-shaped metallic flanges of metal different from the metal of the backing member welded to the backing member with one leg of each flange extending generally at right angles to a face of the backing member and having its extremity butting against said face and with the other legs of the flanges extending toward each other and a metallic facing member disposed against said face of the backing member between the first mentioned legs of the flanges with the second mentioned legs of the flanges overlying a minor portion thereof and held in place against the backing member by the second mentioned legs of the flanges.

held in place against the backing member by the flanges.

5. A composite billet comprising a metallic backing member, opposed generally L-shaped flanges positioned parallel to but spaced inwardly from opposed edges of the backing member with one leg of each flange extending generally at right angles to a face of the backing member and having its extremity butting against said face and with the other legs of the flanges extending toward each other, fillet welds disposed in the corners defined by the outer faces of the first mentioned flange legs and the portions of said face of the backing member disposed between the flanges and the edges of the backing member whereby the flanges are fastened to the backing member and a metallic facing member disposed against said face of the backing member between the first mentioned legs of the flanges with the second mentioned legs of the flanges overlying a minor portion thereof and held in place against the backing member by the flanges.

6. A composite billet comprising a metallic backing member, opposed generally L-shaped flanges positioned at opposed edges of the backing member with one leg of each flange extending generally at right angles to a face of the backing member and having its extremity butting against said face and with the other legs of the flanges extending toward each other, flush welds connecting the outer face of the first mentioned flange legs with the sides of the backing member whereby the flanges are fastened to the backing member and a metallic facing member disposed against said face of the backing member between the first mentioned legs of the flanges with the second mentioned legs of the flanges overlying a minor portion thereof and held in place against the backing member by the flanges.

7. A method of making a composite billet comprising welding to a metallic backing member opposed generally L-shaped flanges with one leg of each flange extending generally at right angles to a face of the backing member and having its extremity butting against said face and with the other legs of the flanges extending toward each

other, then positioning a metallic facing member against said face of the backing member with its edges between said face of the backing member and the second mentioned flange legs and pressing the second mentioned flange legs against the facing member to hold the facing member against said face of the backing member.

8. A method of making a composite billet comprising welding to a metallic backing member opposed generally L-shaped flanges with one leg of each flange extending generally at right angles to a face of the backing member and having its extremity butting against said face and with the other legs of the flanges extending toward each other, then positioning against said face of the backing member with its edges between said face of the backing member and the second mentioned flange legs a metallic facing member narrower than the space between the first mentioned flange legs, laterally positioning the facing member so that there is a substantial space between it and at least one of the first mentioned flange legs and pressing the second mentioned flange legs against the facing member to hold the facing member against said face of the backing member.

WALTER L. KEENE.  
WILLIAM A. CARLSON.

## REFERENCES CITED

30 The following references are of record in the file of this patent:

## UNITED STATES PATENTS

| Number       | Name        | Date           |
|--------------|-------------|----------------|
| 346,661      | Knight      | Aug. 3, 1886   |
| 785,979      | Schmidt     | Mar. 28, 1905  |
| 2,131,115    | Naisuler    | Sept. 27, 1938 |
| 729,113      | Anderson    | May 26, 1903   |
| 976,455      | Grey et al. | Nov. 22, 1910  |
| 40 685,758   | Griffith    | Nov. 5, 1901   |
| 1,886,615    | Johnson     | Nov. 8, 1932   |
| 1,956,818    | Acre        | May 1, 1934    |
| 2,145,248    | Chace       | Jan. 31, 1939  |
| 1,886,615    | Johnson     | Nov. 8, 1932   |
| 45 2,018,725 | Johnson     | Oct. 29, 1935  |
| 2,059,584    | Johnson     | Nov. 3, 1936   |